

## [54] RECORDING MEDIUM FOR SUBLIMATION TYPE HEAT-SENSITIVE TRANSFER RECORDING PROCESS

[75] Inventors: Kenji Kushi; Takayuki Iseki; Tadayuki Fujiwara; Kazuhiko Jufuku; Akifumi Ueda, all of Hiroshima, Japan

[73] Assignee: Mitsubishi Rayon Co., Ltd., Tokyo, Japan

[21] Appl. No.: 22,296

[22] Filed: Feb. 25, 1993

## [30] Foreign Application Priority Data

|                    |             |          |
|--------------------|-------------|----------|
| Feb. 27, 1992 [JP] | Japan ..... | 4-041741 |
| Feb. 27, 1992 [JP] | Japan ..... | 4-041742 |
| Oct. 23, 1992 [JP] | Japan ..... | 4-286399 |
| Oct. 26, 1992 [JP] | Japan ..... | 4-287982 |
| Nov. 5, 1992 [JP]  | Japan ..... | 4-295791 |
| Dec. 28, 1992 [JP] | Japan ..... | 4-348725 |

[51] Int. Cl.<sup>5</sup> ..... B41M 5/035; B41M 5/38

[52] U.S. Cl. ..... 503/227; 428/195; 428/480; 428/704; 428/913; 428/914

[58] Field of Search ..... 8/471; 428/195, 913, 428/914, 480, 704; 503/227

## [56] References Cited

## U.S. PATENT DOCUMENTS

|                                       |         |
|---------------------------------------|---------|
| 4,778,782 10/1988 Ito et al. ....     | 503/227 |
| 5,185,316 2/1993 Egashira et al. .... | 503/227 |

## FOREIGN PATENT DOCUMENTS

|                                        |         |
|----------------------------------------|---------|
| 0261505 3/1988 European Pat. Off. .... | 503/227 |
| 0431184 6/1991 European Pat. Off. .... | 503/227 |
| 61-229594 10/1986 Japan ....           | 503/227 |
| 62-46689 2/1987 Japan ....             | 503/227 |
| 63-67188 3/1988 Japan ....             | 503/227 |
| 1-127387 5/1989 Japan ....             | 503/227 |
| 1-171887 7/1989 Japan ....             | 503/227 |
| 3-19893 1/1991 Japan ....              | 503/227 |

Primary Examiner—B. Hamilton Hess

Attorney, Agent, or Firm—Oblon, Spivak, McClelland, Maier & Neustadt

## [57] ABSTRACT

A recording medium for sublimation type heat-sensitive transfer recording process, in which an image receiving layer comprising a resin composition containing a dyeable resin and at least one phosphite antioxidant shown in Formulas (1), (2), or (3) is formed on a substrate surface. This recording medium for sublimation type heat-sensitive recording methods has extremely superior light resistance, and the image recorded on this

recording medium suffers little fade out or discoloration as a result of exposure to light, so that this recording medium is expected to contribute greatly to the spread of video printers and the like.



(In Formula (1), R<sub>1</sub> and R<sub>2</sub> represent H or an alkyl group having a number of carbon atoms within a range of 1-20, R<sub>3</sub> and R<sub>4</sub> represent alkyl groups having a number of carbon atoms within a range of 1-20, X represents H or an atomic group having 1-10 carbon atoms as a main skeleton thereof, and n has a value of 1, 2, 3, or 4.)



(In Formula (2), R<sub>5</sub> and R<sub>6</sub> represent H or an alkyl group having a number of carbon atoms within a range of 1-20, R<sub>7</sub> represents an alkyl group having a number of carbon atoms within a range of 1-20, Y represents H or an atomic group having 1-10 carbon atoms as a main skeleton thereof, and n has a value of 1, 2, 3, or 4.)



(In Formula (3), R<sub>8</sub>, R<sub>9</sub>, R<sub>10</sub>, and R<sub>11</sub> represent H or an alkyl group having a number of carbon atoms within a range of 1-20, Z represents H or an atomic group having 1-10 carbon atoms as a main skeleton thereof, and n has a value of 1, 2, 3, or 4.)

21 Claims, No Drawings

RECORDING MEDIUM FOR SUBLIMATION  
TYPE HEAT-SENSITIVE TRANSFER RECORDING  
PROCESS

BACKGROUND OF THE INVENTION

1. Field of the Invention

The present invention relates to a recording medium for sublimation type heat-sensitive transfer recording process which forms a recorded image which has superior resistance to fading when exposed to light. 10

2. Background Art

Sublimation type heat-sensitive transfer recording process are advantageous in that the level of noise produced during recording is low, the apparatus used therefor is small and inexpensive, the maintenance thereof is easy, and the output time is short. Furthermore, since sublimation type dyes are used, by continuously varying the amount of the exothermic energy, high contrast recording may be easily achieved, and such recording exhibits high density and high resolution. As a result, in comparison with other recording methods, such a method is advantageous, especially for 15 producing full color hard copy, and has been adopted as a recording method for color printers, video printers, and the like.

However, as the image recorded by means of such a sublimation type heat-sensitive transfer recording process is formed by means of sublimable dyes, the light 20 resistance thereof is generally poor, and this is disadvantageous in that fade out and discoloration resulting from sunlight or fluorescent light exposure occurs easily. In order to solve this problem, an ultraviolet absorber or a 25 photostabilizer was generally applied to the image receiving layer of the recording medium, and as a result of this, light resistance was somewhat improved; however, this improvement could not be termed sufficient. In addition, methods have been disclosed, such as that in Japanese Laid-Open Patent Application No. Hei 1-127387, in which a specified phenol antioxidant was 30 applied to the image receiving layer, and that of Japanese Laid-Open Patent Application No. Hei 3-19893, and Japanese Laid-Open Patent Application No. Sho 61-229594, in which a specified phosphorus antioxidant was applied to the image receiving layer, and as a result of using these methods, a small increase in light resistance was observed; however, the degree of fade out 35 and discoloration as a result of exposure to light was still large. 40

SUMMARY OF THE INVENTION

It is an object of the present invention to provide a recording medium for a sublimation type heat-sensitive transfer recording process, the image recorded thereon having superior resistance to light exposure, and which exhibits a very low level of fade out and discoloration resulting from exposure to light. 45

The recording medium for sublimation type heat-sensitive transfer recording process in accordance with the present invention has formed, on the substrate surface thereof, an image receiving layer comprising a resin composition containing at least one of the phosphite antioxidants shown in Formulas (1), (2), and (3) below, and a dyeable resin. 50

5

2



(In Formula (1), R<sub>1</sub> and R<sub>2</sub> represent H or an alkyl group having a number of carbon atoms within a range of 1-20, R<sub>3</sub> and R<sub>4</sub> represent an alkyl group having a number of carbon atoms within a range of 1-20, X represents H or an atomic group having 1-10 carbon atoms as a main skeleton thereof, and n has a value of 1, 2, 3, or 4.)

15



20

(In Formula (2), R<sub>5</sub> and R<sub>6</sub> represent H or an alkyl group having a number of carbon atoms within a range of 1-20, R<sub>7</sub> represents an alkyl group having a number of carbon atoms within a range of 1-20, Y represents H or an atomic group having 1-10 carbon atoms as a main skeleton thereof, and n has a value of 1, 2, 3, or 4.)

25



30

(In Formula (3), R<sub>8</sub>, R<sub>9</sub>, R<sub>10</sub>, and R<sub>11</sub> represent H or an alkyl group having a number of carbon atoms within a range of 1-20, Z represents H or an atomic group having 1-10 carbon atoms as a main skeleton thereof, and n has a value of 1, 2, 3, or 4.)

35

Furthermore, in accordance with the recording medium for sublimation type heat-sensitive transfer recording process in accordance with the present invention, by means of including a phosphite antioxidant having the specified structure in the image receiving layer, the light resistance is greatly increased, and the image which is recorded on this recording medium exhibits extremely low levels of fade out and discoloration resulting from exposure to light, so that this recording medium is expected to contribute greatly to the wider use of video printers, and the like. 40

45

50

55

60

DETAILED DESCRIPTION OF THE  
INVENTION

Examples of the substrate constituting the recording medium in accordance with the present invention include films or papers, for example, various plastic films, such as polyester film, polyethylene film, polypropylene film, polystyrene film, nylon film, vinyl chloride

film, and the like or white films in which white pigment or filler has been added to one of these films; examples of papers include papers having cellulose fibers as the main component thereof such as recording paper, art paper, coated paper, and the like, and papers having plastic fibers as the main component thereof such as acrylic paper, polypropylene paper, polyester paper, and the like. These papers or films may be used without being subjected to preprocessing, or where necessary, preprocessing such as washing, etching, corona discharge, activating energy irradiation, dyeing, printing, or the like, may be carried out prior to use. Furthermore, a laminated substrate, in which two or more of the above substrates are laminated together, may also be used. The thickness of the substrate is not particularly restricted; however, a thickness in a range of 20-500 micrometers is preferable.

An image receiving layer is formed on at least one surface of the above substrate; this image receiving layer receives and develops the sublimable dye which is transferred from the transfer sheet. The medium constituting this image receiving layer is not particularly restricted, insofar as the medium is easily dyed by means of sublimable dyes, and does not cause blocking of the transfer sheet during recording; examples of such a medium include cellulose resins, such as methyl cellulose, ethyl cellulose, ethyl hydroxy cellulose, hydroxy ethyl cellulose, hydroxy propyl cellulose, cellulose acetate, and the like; vinyl resins such as polyvinyl alcohol, polyvinyl butylal, polyvinyl acetal, polyvinyl acetate, polyvinyl chloride, polyvinyl pyrrolidone, styrene, and the like; acrylate resins, such as polymethyl (meth)acrylate, polybutyl (meth)acrylate, polyacrylamide, polyacrylonitrile, and the like; furthermore, polyester resin, polycarbonate resin, polyurethane resin, polyamide resin, urea resin, polycaprolactone resin, polyallylate resin, polysulfone resin, or copolymers or mixtures thereof, can be used as dyable resins. Among these, polyester resin is easily dyed by means of sublimable dyes, and the image obtained has good storage stability, so that it is preferable that polyester resin be included as at least one component of the dyeable resin.

It is preferable to include a cross-linking component in the image receiving layer in accordance with the present invention, in order to increase the separability of the image receiving layer from the transfer sheet. For example, it is possible to include heat curable components such as isocyanate and polyol and the like, and to thermally cross-link these components after the formation of the image receiving layer, or to apply a cross-linking agent curable by means of activating energy rays, for example, a resin composition including monomers or oligomers possessing acryloyloxy groups or methacryloyloxy groups, to the surface of a substrate, and then to cure this by means of activating energy rays, thus yielding an image receiving layer. In particular, in the case of a method in which components which can be cross-linked by means of activated energy rays are blended, cured by means of activating energy rays, and an image receiving layer thus obtained, high productivity becomes possible, the surface gloss of the resulting image receiving layer is high, and the storage stability of the recorded image with respect to heat is high, so that such a method is more preferable.

The amount of the above dyeable resin and cross-linking components which are used are not particularly restricted; however, it is preferable that, with respect to a total amount of both the dyeable resin and the cross-

linking components of 100 parts by weight, the dyeable resin be present in an amount of 40-95 parts by weight, while the cross-linking components be present in an amount of 60-5 parts by weight.

The resin composition containing a cross-linking agent curable by means of activating energy rays may be cured by activating energy rays such as an electron beam or ultraviolet radiation; however, in the case in which ultraviolet radiation is used as the activating energy rays, it is desirable to include a conventional photopolymerization initiator. The amount of photopolymerization initiator which is used is not particularly restricted; however, it is preferable that, with respect to a total amount of the above-described dyeable resin forming the image receiving layer and cross-linking components of 100 parts by weight, the photopolymerization initiator be present in an amount of 0.1-10 parts by weight.

In the present invention, in order to achieve an increase in the photoresistance of the image recorded on the image receiving layer, the most important condition is the inclusion, as stated above, of at least one of the phosphite antioxidants, shown in the Formulas (1), (2), and (3) below, in the resin composition forming the image receiving layer.



(In Formula (1), R<sub>1</sub> and R<sub>2</sub> represent H or an alkyl group having a number of carbon atoms within a range of 1-20, R<sub>3</sub> and R<sub>4</sub> represent alkyl groups having a number of carbon atoms within a range of 1-20, X represents H or an atomic group having 1-10 carbon atoms as a main skeleton thereof, and n has a value of 1, 2, 3, or 4.)



(In Formula (2), R<sub>5</sub> and R<sub>6</sub> represent H or an alkyl group having a number of carbon atoms within a range of 1-20, R<sub>7</sub> represents alkyl groups having a number of carbon atoms within a range of 1-20, Y represents H or an atomic group having 1-10 carbon atoms as a main skeleton thereof, and n has a value of 1, 2, 3, or 4.)



(In Formula (3), RS, R<sub>9</sub>, R<sub>10</sub>, and R<sub>11</sub> represent H or an alkyl group having a number of carbon atoms within a range of 1-20, represents H or an atomic group having 1-10 carbon atoms as a main skeleton thereof, and n has a value of 1, 2, 3, or 4.)

By means of blending a phosphite antioxidant compound possessing the specified structure described above into the resin composition forming the image receiving layer, the light resistance of the recorded image increases to an unexpected extent, in comparison with conventional resin compositions, and the fade out and discoloration resulting from exposure to light becomes extremely small.

The compounds shown in the following Structural Formulas (A)-(I) below are concrete examples of the phosphite antioxidant shown in Formulas (1), (2), and (3).

(3)

5

10

-continued

(G)



(H)



(I)



It is possible to use these phosphite antioxidants singly or in a mixture of two or more. The amounts of these antioxidants which are used are not particularly restricted; however, with respect to 100 parts by weight of the dyeable resin or 100 parts by weight of the dyeable resin and cross-linking components which form the image receiving layer, respectively, it is preferable that this antioxidant be present in an amount of 0.3-20 parts by weight, and more preferably in an amount of 1-15 parts by weight. If the amount used is too small, it is difficult to obtain the superior light resistance which is an object of the present invention, while when the amount used is too great, the antioxidant easily bleeds out of the surface of the image receiving layer, and the recorded image blurs easily over time.

(A)



(B)



(R = an alkyl group having a number of carbon atoms within a range of 12-15)

(C)



(D)



(E)



(F)



(In Formula (4), R<sub>12</sub>, R<sub>13</sub>, and R<sub>14</sub> represent H or an alkyl group having a number of carbon atoms within a range of 1-4.)

By using a phenol compound having the specified structure shown in the above Formula (4), instead of a hindered phenol antioxidant disclosed in Japanese Laid-Open Patent Application No. Hei 1-127387, it was discovered that the light resistance of the recorded image was further increased, and fade out and discoloration resulting from exposure to light were further reduced, as stated above.

Moreover, by adding a phenol compound possessing the specified structure shown in Formula (4) above, it was discovered that not merely does light resistance increase, but recording density becomes high, and resistance to dark fade-out (resistance to discoloration or reduction in density when a recorded image is stored for long periods at high temperatures) is also increased.

The compounds shown in Structural Formula (J) below are concrete examples of the phenol compound shown in Formula (4).





(J)

The phenol compound shown in Formula (4) may be used singly, or two or more variants thereof may be mixed and used. The amounts of these phenol compounds which are used are not particularly restricted; however, with respect to a total of 100 parts by weight of dyeable resin constituting the image receiving layer, or with respect to a total of 100 parts by weight of dyeable resin and cross-linking components constituting the image receiving layer, it is preferable that this phenol compound be present in an amount of 0.3-20 parts by weight, and preferably in an amount of 1-15 parts by weight. If the amount used thereof is too small, the superior light resistance which is an object of the present invention is difficult to obtain, and furthermore, there is a tendency for the effect of an increase in the dyeing density and the effect of an increase in the resistance to dark fade-out to be insufficient. When the amount used thereof is too great, the compound easily bleeds out onto the surface of the image receiving layer, and the recorded image thus tends to blur over time.

In the present invention, in order to further increase the light resistance of the image receiving layer, it is permissible to include an ultraviolet absorber in addition to the phosphite antioxidants shown in Formulas (1)-(3) and the compounds shown in Formula (4) above.

It is possible to use conventional ultraviolet absorbers such as benzotriazole ultraviolet absorbers or benzophenone ultraviolet absorbers, or the like, as these ultraviolet absorbers. Concrete examples of benzotriazole ultraviolet absorbers include, for example, 2-(5-methyl-2-hydroxy phenyl) benzotriazole (manufactured by Ciba-Geigy: TINUVIN P), 2-[2-hydroxy-3,5-bis( $\alpha$ , $\alpha$ -dimethyl-benzyl) phenyl]-2H-benzotriazole (manufactured by Ciba-Geigy: TINUVIN 234), 2-(5-t-butyl-2-hydroxy phenyl) benzotriazole (manufactured by Ciba-Geigy: TINUVIN PS), 2-(3,5-di-t-butyl-2-hydroxy phenyl) benzotriazole (manufactured by Ciba-Geigy: TINUVIN 320), 2-(3-t-butyl-5-methyl-2-hydroxy phenyl)-5-chlorobenzotriazole (manufactured by Ciba-Geigy: TINUVIN 326), 2-(3,5-di-t-butyl-2-hydroxyphenyl)-5-chlorobenzotriazole (manufactured by Ciba-Geigy: TINUVIN 327), 2-(3,5-di-t-amyl-2-hydroxy phenyl) benzotriazole (manufactured by Ciba-Geigy: TINUVIN 328), 2-[2-hydroxy-3-(3,4,5,6-tetrahydrophthalimide methyl)-5-methyl phenyl] benzotriazole (manufactured by Sumitomo Chemical Company, Limited: SUMISORB 250), 2-(4-octoxy-2-hydroxyphenyl) benzotriazole, and the like. Concrete examples of the benzophenone ultraviolet absorber include, for example, 2,4-dihydroxybenzophenone, 2-hydroxy-4-methoxy benzophenone, 2-hydroxy-4-octoxybenzophenone, 2-hydroxy-4-dodecyloxybenzophenone, 2-hydroxy-4-benzoyloxybenzophenone, 2,2'-dihydroxy-4-methoxy benzophenone, 2,2'4,4'-tetrahydroxy benzophenone, 2,2'-dihydroxy-4,4'-dimethoxybenzophenone, 2,2'-dihydroxy-4,4'-dioctoxy benzophenone, 2,2'-dihydroxy-4,4'-didodecyloxy benzophenone, 2-hydroxy-4-methoxy-5-sulfobenzophenone, and the like.

These ultraviolet absorbers may be used singly or in a mixture of two or more thereof. The amounts used thereof are not particularly restricted; however, with respect to a total of 100 parts by weight of dyeable resin,

or with respect to a total of 100 parts by weight of dyeable resin and cross-linking components, the ultraviolet absorber may be preferably present in an amount of 1-10 parts by weight. If the amount used is too small, the effect of an increase in light resistance is insufficient, while when the amount used is too great, the ultraviolet absorber bleeds onto the surface of the image receiving layer, and the recorded image tends to blur over time.

Furthermore, in order to further increase the light resistance of the image receiving layer, it is acceptable to include a hindered amine photostabilizer in the resin composition forming the image receiving layer. Conventional hindered amine photostabilizers may be used; concrete examples thereof include, for example, bis(2,2,6,6-tetramethyl-4-piperidyl) sebacate (manufactured by Sankyo Company, Limited: SANOL LS770), bis(1,2,2,6,6-pentamethyl-4-piperidyl) sebacate (manufactured by Sankyo Company, Limited: SANOL LS765), 1-[2-[3-(3,5-di-t-butyl-4-hydroxy phenyl) propionyloxy] ethyl]-4-[3-(3,5-di-t-butyl-4-hydroxy phenyl) propionyloxy]-2,2,6,6-tetramethyl piperidine (manufactured by Sankyo Company, Limited: SANOL LS2626), 4-benzoyloxy-2,2,6,6-tetramethyl piperidine (manufactured by Sankyo Company, Limited: SANOL LS744), 8-acetyl-3-dodecyl-7,7,9,9-tetramethyl-1,3,8-triaza-spiro [4,5] decane-2,4-dione (manufactured by Sankyo Company, Limited: SANOL LS440), 2-(3,5-di-t-butyl-4-hydroxy benzyl)-2-n-butylmalonate bis (1,2,2,6,6-pentamethyl-4-piperidyl) (manufactured by Ciba-Geigy: TINUVIN 144), succinate bis (2,2,6,6-tetramethyl-4-piperidinyl) ester (manufactured by Ciba-Geigy: TINUVIN 780 FF), a condensation polymer of dimethyl succinate and 1-(2-hydroxy ethyl)-4-hydroxy-2,2,6,6-tetramethyl piperidine (manufactured by Ciba-Geigy: TINUVIN 622 LD), poly{[6-(1,1,3,3-tetramethylbutyl) amino-1,3,5-triazine-2,4-dyl][(2,2,6,6-tetramethyl-4-piperidyl) imino] hexamethylene [(2,2,6,6-tetramethyl-4-piperidyl) imino]} (manufactured by Ciba-Geigy: CHIMASSORB 944LD), a condensation polymer of N,N'-bis(3-aminopropyl) ethylene diamine and 2,4-bis [N-butyl-N-(1,2,2,6,6-pentamethyl-4-piperidyl) amino]-6-chloro-1,3,5-triazine (manufactured by Ciba-Geigy: CHIMASSORB 119FL), HA-70G (manufactured by Sankyo Company, Limited), ADK STAB LA-52, ADK STAB LA-57, ADK STAB LA-62, ADK STAB LA-67, ADK STAB LA-63, ADK STAB LA-68, ADK STAB LA-82, ADK STAB LA-87 (all produced by Asahi Denka Kogyo K.K.), and the like.

These hindered amine photostabilizers may be used singly or in a mixture of two or more; however, when the effect of an increase in light resistance is taken into account, it is preferable that they be used in concert with the above-described ultraviolet absorbers. The amounts used of these hindered amine photostabilizers is not particularly restricted; however, with a respect to a total of 100 parts by weight of dyeable resin, or with respect to a total of 100 parts by weight of dyeable resin and cross-linking components, it is preferable that the hindered amine photostabilizer be present in an amount of 1-10 parts by weight. If the amount used is too small, the effect of an increase in light resistance cannot be sufficiently attained, while on the other hand, when the amount used is too large, the hindered amine photostabilizer tends to bleed out onto the surface of the image receiving layer, and thus the recorded image tends to blur over time.

Furthermore, it is permissible to include a releasing agent in the image receiving layer in accordance with the present invention in order to further increase the separability of the image receiving layer from the transfer sheet. Examples of this releasing agent include silicone surfactants, fluorine surfactants, a graft polymer using polyorganosiloxane as a trunk or a branch, silicon or fluorine compounds producible a cross-linked structure, for example, a combination of amino-denatured silicon and epoxy-denatured silicon, and the like; the releasing agents may be used singly or concurrently. The amount of the releasing agent used is not particularly restricted; however, with respect to a total of 100 parts by weight of dyeable resin, or with respect to a total of 100 parts by weight of dyeable resin and cross-linking components, it is preferable that the releasing agent be present in an amount of 0.01-30 parts by weight.

Furthermore, depending on the purpose of use, inorganic fillers such as silica, calcium carbonate, titanium oxide, zinc oxide, and the like, may be included in the above resin compositions.

In manufacturing the recording medium of the present invention, the resin composition may be applied directly to a substrate surface by means of a coating method such as roll coating, bar coating, blade coating, or the like, and the image receiving layer can thus be formed. However, in order to increase the efficiency of the application process, the resin composition may be blended with a solvent able to dissolve the resin composition, such as, for example, ethyl alcohol, methylethylketone, toluene, ethyl acetate, dimethyl formamide, tetrahydrofuran, and the like, and appropriate adjustment of the application viscosity may be carried out. By means of this, application may easily be conducted by means of spray coating, curtain coating, flow coating, dip coating, or the like. In the case in which such solvents are blended with the resin composition, the solvents must be volatilized and dried after the coating of the resin composition.

The image receiving layer preferably have a thickness of 0.5-100 micrometers, and more preferably within a range of 1-50 micrometers. At a thickness of less than 0.5 micrometers, the high recording density will not be easily obtained.

Furthermore, the recording medium in accordance with the present invention may have a layer such as an adhesion facilitating layer, an electrostatic prevention layer, a whiteness improving layer, or a compound layer combining these functions provided between the image receiving layer and the substrate. In addition, in this recording medium in accordance with the present invention, processing such as electrostatic prevention processing, contaminant protection processing, smoothing processing, and writing facilitation processing may be carried out on the side opposite the image receiving layer.

### EXAMPLES

Hereinbelow, the present invention will be explained in detail based on examples.

In the following Examples and Comparative Examples, part(s) means part(s) by weight, respectively.

### EXAMPLE 1

On one side of a sheet of art paper (thickness 85 micrometers), a white polyester film (manufactured by Diafoil Hoechst: W900, thickness 38 micrometers) was

laminated, and on the other side of this paper, a sheet of white polypropylene paper (manufactured by Oji Yuka: Yupo FPG, thickness 60 micrometers) was laminated, and a substrate was thus obtained. The AD-577-1 and the CAT-52 adhesives produced by Toyo Morton Co., Ltd. were used as the adhesives therefor.

The coating fluid for the image receiving layer described hereinbelow was coated uniformly to the surface of the white polyester film of the substrate thus obtained, by means of an immersion method, and after the volatilization of the solvent, this was irradiated with ultraviolet rays by means of a high pressure mercury lamp, and an image receiving layer having a thickness of 5-6 micrometers was formed, so that a recording medium was obtained.

#### Coating Fluid for Image Receiving Layer

|                                                                                                                                                                                                                                                                                                         |           |
|---------------------------------------------------------------------------------------------------------------------------------------------------------------------------------------------------------------------------------------------------------------------------------------------------------|-----------|
| Polyester resin formed from the condensation polymerization of terephthalic acid/isophthalic acid/ethylene glycol/neopentyl glycol (molecular weight 15000-20000, glass transition temperature 67° C.)                                                                                                  | 20 parts  |
| Polyester resin formed from the condensation polymerization of terephthalic acid/isophthalic acid/sebacic acid/ethylene glycol/neopentyl glycol/1,4-butane diol (molecular weight 18000-20000, glass transition temperature 47° C.)                                                                     | 50 parts  |
| Kayarad DPHA (produced by Nippon Kayaku Co., Ltd)                                                                                                                                                                                                                                                       | 15 parts  |
| 2,2-bis(4-acryloxyloxy diethoxy phenyl) propane                                                                                                                                                                                                                                                         | 15 parts  |
| 1-hydroxycyclohexylphenyl ketone                                                                                                                                                                                                                                                                        | 3 parts   |
| Phosphite antioxidant expressed in Structural Formula (A) above (produced by Asahi Denka Kogyo K.K.: ADK STAB 517)                                                                                                                                                                                      | 8.0 parts |
| 2-hydroxy-4-octoxybenzophenone                                                                                                                                                                                                                                                                          | 4.8 parts |
| Bis(1,2,2,6,6-pentamethyl-4-piperidyl) sebacate                                                                                                                                                                                                                                                         | 4.8 parts |
| Silicone surfactant expressed in Structural Formula (5) below                                                                                                                                                                                                                                           | 0.5 parts |
| $(5) \quad \begin{array}{c} \text{CH}_3 & \text{CH}_3 & \text{CH}_3 \\   &   &   \\ \text{CH}_3-\text{Si}(\text{O})-\text{Si}(\text{O})_m-\text{Si}-\text{CH}_3 \\   &   &   \\ \text{CH}_3 & \text{O} & \text{CH}_3 \\   & &   \\ (\text{C}_2\text{H}_4\text{O})_x-\text{COC}_2\text{H}_5 \end{array}$ |           |
| $\left( \frac{2l+m+1}{mx} = 1.3 \right)$                                                                                                                                                                                                                                                                |           |
| Methylethyl ketone                                                                                                                                                                                                                                                                                      | 500 parts |
| toluene                                                                                                                                                                                                                                                                                                 | 100 parts |

The recording medium which was thus obtained was used for recording using the cyan color of the color sheet VW-VS 100 for the NV-MP1 video printer produced by Matsushita Electric Industrial Co., Ltd., and using a thermal head produced by Kyocera Corporation (950 Ohms, 6 dots/mm) and under conditions such that the recording voltage was 13 V, and the pulse width was 10 msec. Subsequently, the recorded image was exposed for a period of 72 hours using a xenon long life fade meter (produced by Suga Test Instruments Co., Ltd.: model FAL-25AX) and the color variation ( $\Delta E$ ) before and after exposure was measured. The results thereof are shown in Table 1.

### EXAMPLE 2

In Example 2, a process was followed which was identical to that of Example 1, with the exception that in place of the phosphite antioxidant (A) (ADK STAB 517), 8.0 parts of the phosphite antioxidant expressed in

Structural Formula (B) above (produced by Asahi Denka Kogyo K.K.: ADK STAB 1500) was used, and a recording medium was obtained.

The recording medium which was thus obtained was tested in the same manner as in Example 1, and  $\Delta E$  was measured. The results thereof are shown in Table 1.

### EXAMPLE 3

In Example 3, a process was followed which was identical to that of Example 1, with the exception that in place of the phosphite antioxidant (A) (ADK STAB 517) which was used in Example 1, 8.0 parts of the phosphite antioxidant expressed in Structural Formula (C) above (produced by Asahi Denka Kogyo K.K.: ADK STAB 260) was used, and a recording medium was obtained.

The recording medium which was thus obtained was tested in the same manner as in Example 1, and  $\Delta E$  was measured. The results thereof are shown in Table 1.

### EXAMPLE 4

In Example 4, a process was followed which was identical to that of Example 1, with the exception that in place of the phosphite antioxidant (A) (ADK STAB 517) which was used in Example 1, 8.0 parts of the phosphite antioxidant expressed in Structural Formula (D) (produced by Asahi Denka Kogyo K.K.: ADK STAB 522A) was used, and a recording medium was obtained.

The recording medium which was thus obtained was tested in the same manner as in Example 1, and  $\Delta E$  was measured. The results thereof are shown in Table 1.

### EXAMPLE 5

In Example 5, a process was followed which was identical to that of Example 1, with the exception that in place of the phosphite antioxidant (A) (ADK STAB 517) which was used in Example 1, 8.0 parts of the phosphite antioxidant expressed in Structural Formula (E) (produced by Johoku Chemical Co., Ltd.: JPP-613M) was used, and a recording medium was obtained.

The recording medium which was thus obtained was tested in the same manner as in Example 1, and  $\Delta E$  was measured. The results thereof are shown in Table 1.

### EXAMPLE 6

In Example 6, a process was followed which was identical to that of Example 1, with the exception that the amount of the phosphite antioxidant (A) (ADK STAB 517) which was used was set at 1.6 parts.

The recording medium which was thus obtained was tested in the same manner as in Example 1, and  $\Delta E$  was measured. The results thereof are shown in Table 1.

### EXAMPLE 7

In Example 7, a process was followed which was identical to that of Example 1, with the exception that the amount of the phosphite antioxidant (A) (ADK STAB 517) which was used was set at a level of 3.2 parts.

The recording medium which was thus obtained was tested in the same manner as in Example 1, and  $\Delta E$  was measured. The results thereof are shown in Table 1.

### EXAMPLE 8

In Example 8, a process was followed which was identical to that of Example 1, with the exception that in place of the two types of polyester resin which were

used in Example 1, 70 parts of a polyester resin obtained by the condensation polymerization of terephthalic acid/isophthalic acid/ethylene glycol/neopentyl glycol/1,4-cyclohexane dimethanol (molecular weight 25,000-30,000, glass transition temperature 67°C.) was used, and the amount of the phosphite antioxidant (A) (ADK STAB 517) which was used was set at a level of 4.8 parts, and a recording medium was obtained.

The recording medium which was thus obtained was tested in the same manner as in Example 1, and  $\Delta E$  was measured. The results thereof are shown in Table 1.

### EXAMPLE 9

In Example 9, a process was followed which was identical to that of Example 8, with the exception that the amount of the phosphite antioxidant (A) (ADK STAB 517) which was used was set at a level of 13.0 parts, and a recording medium was obtained.

The recording medium which was thus obtained was tested in the same manner as in Example 1, and  $\Delta E$  was measured. The results thereof are shown in Table 1.

### EXAMPLE 10

The coating fluid for the image receiving layer described hereinbelow was uniformly coated to the surface of white polyester film constituting the substrate used in Example 1, by means of an immersion method, and the solvent was volatilized, and subsequently, this was heated for a period of 2 hours at a temperature of 100°C., and an image receiving layer having a thickness of 5-6 micrometers was formed, so that a recording medium was obtained.

| Coating Fluid for the Image Receiving Layer                                                                                                                                                                                      |            |
|----------------------------------------------------------------------------------------------------------------------------------------------------------------------------------------------------------------------------------|------------|
| Polyester resin formed by the condensation polymerization of terephthalic acid/isophthalic acid/ethylene glycol/neopentyl glycol (molecular weight 15000-20000, glass transition temperature 67°C.)                              | 24 parts   |
| Polyester resin formed by the condensation polymerization of terephthalic acid/isophthalic acid/sebacic acid/ethylene glycol/neopentyl glycol/1,4-butane diol (molecular weight 18000-20000, glass transition temperature 47°C.) | 60 parts   |
| Amino-denatured silicone oil (produced by Shin-Etsu Chemical Co., Ltd.: KF-393)                                                                                                                                                  | 8 parts    |
| Epoxy-denatured silicone oil (produced by Shin-Etsu Chemical Co., Ltd.: X-22-343)                                                                                                                                                | 8 parts    |
| Phosphite antioxidant expressed by Structural Formula (A) above (produced by Asahi Denka Kogyo K.K.: ADK STAB 517)                                                                                                               | 11.3 parts |
| Methylethyl ketone                                                                                                                                                                                                               | 300 parts  |
| Toluene                                                                                                                                                                                                                          | 300 parts  |

The recording medium which was obtained was tested in the same manner as in Example 1, and  $\Delta E$  was measured. The results are shown in Table 1.

### EXAMPLE 11

In Example 11, a process was followed which was identical to that of Example 1, with the exception that in place of the phosphite antioxidant (A) (ADK STAB 517) which was used in Example 1, 8.0 parts of the phosphite antioxidant expressed by Structural Formula (F) (produced by Asahi Denka Kogyo K.K.: ADK STAB C) was used, and a recording medium was obtained.

The recording medium which was thus obtained was tested in the same manner as in Example 1, and  $\Delta E$  was measured. The results thereof are shown in Table 1.

#### EXAMPLE 12

In Example 12, a process was followed which was identical to that of Example 1, with the exception in place of the phosphite antioxidant (A) (ADK STAB 517) which was used in Example 1, 8.0 parts of the phosphite antioxidant expressed by Structural Formula (G) above (produced by Johoku Chemical Co., Ltd.: JPM-311) was used, and a recording medium was obtained.

The recording medium which was thus obtained was tested in the same manner as in Example 1, and  $\Delta E$  was measured. The results thereof are shown in Table 1.

#### EXAMPLE 13

In Example 13, a process was followed which was identical to that of Example 1, with the exception that in place of the phosphite antioxidant (A) (ADK STAB 517) which was used in Example 1, 8.0 parts of the phosphite antioxidant expressed by Structural Formula (H) above (produced by Johoku Chemical Co., Ltd.: JPM-313) was used, and a recording medium was obtained.

The recording medium which was thus obtained was tested in the same manner as in Example 1, and  $\Delta E$  was measured. The results thereof are shown in Table 1.

#### EXAMPLE 14

In Example 14, a process was followed which was identical to that of Example 1, with the exception that in place of the phosphite antioxidant (A) (ADK STAB 517) which was used in Example 1, 8.0 parts of the phosphite antioxidant expressed by Structural Formula (I) above (produced by Johoku Chemical Co., Ltd.: JPP-100) was used, and a recording medium was obtained.

The recording medium which was thus obtained was tested in the same manner as in Example 1, and  $\Delta E$  was measured. The results thereof are shown in Table 1.

#### EXAMPLE 15

In Example 15, a process was followed which was identical to that of Example 1, with the exception that in place of the phosphite antioxidant (A) (ADK STAB 517) which was used in Example 1, 1.6 parts of the phosphite antioxidant expressed by Structural Formula (F) above (produced by Asahi Denka Kogyo K.K.: ADK STAB C) was used, and a recording medium was obtained.

The recording medium which was thus obtained was tested in the same manner as in Example 1, and  $\Delta E$  was measured. The results thereof are shown in Table 1.

#### EXAMPLE 16

In Example 16, a process was followed which was identical to that of Example 1, with the exception that in place of the phosphite antioxidant (A) (ADK STAB

517) which was used in Example 1, 3.2 parts of the phosphite antioxidant expressed by Structural Formula (F) above (produced by Asahi Denka Kogyo K.K.: ADK STAB C) was used, and a recording medium was obtained.

The recording medium which was thus obtained was tested in the same manner as in Example 1, and  $\Delta E$  was measured. The results thereof are shown in Table 1.

#### EXAMPLE 17

In Example 17, a process was followed which was identical to that of Example 1, with the exception that in place of the phosphite antioxidant (A) (ADK STAB 517) which was used in Example 1, 13.0 parts of the phosphite antioxidant expressed by Structural Formula (F) above (produced by Asahi Denka Kogyo K.K.: ADK STAB C) was used, and a recording medium was obtained.

The recording medium which was thus obtained was tested in the same manner as in Example 1, and  $\Delta E$  was measured. The results thereof are shown in Table 1.

#### EXAMPLE 18

In Example 18, a process was followed which was identical to that of Example 10, with the exception that in place of the phosphite antioxidant (A) (ADK STAB 517) which was used in Example 10, 11.3 parts of the phosphite antioxidant expressed by Structural Formula (F) above (produced by Asahi Denka Kogyo K.K.: ADK STAB C) was used, and a recording medium was obtained.

The recording medium which was thus obtained was tested in the same manner as in Example 1, and  $\Delta E$  was measured. The results thereof are shown in Table 1.

#### Comparative Example 1

In Comparative Example 1, a process was followed which was identical to that of Example 1, with the exception that the phosphite antioxidant (A) (ADK STAB 517) was not used, and a recording medium was obtained.

The recording medium which was thus obtained was tested in the same manner as in Example 1, and  $\Delta E$  was measured. The results thereof are shown in Table 1.

#### Comparative Example 2

In Comparative Example 2, a process was followed which was identical to that of Example 1, with the exception that in place of the phosphite antioxidant (A) (ADK STAB 517) which was used in Example 1, 8.0 parts of the hindered phenone antioxidant expressed by the Structural Formula (6) below (produced by Asahi Denka Kogyo K.K.: ADK STAB AO-75) was used, and a recording medium was obtained.

The recording medium which was thus obtained was tested in the same manner as in Example 1, and  $\Delta E$  was measured. The results thereof are shown in Table 1.



## Comparative Example 3

In Comparative Example 3, a process was followed which was identical to that of Example 1, with the exception that in place of the phosphite antioxidant (A) (ADK STAB 517) which was used in Example 1, 8.0 parts of the hindered phenone antioxidant expressed by the Structural Formula (7) below (produced by Sumitomo Chemical Company, Limited: Sumilizer BP-101) was used, and a recording medium was obtained.

The recording medium which was thus obtained was tested in the same manner as in Example 1, and  $\Delta E$  was measured. The results thereof are shown in Table 1.



## Comparative Example 4

In Comparative Example 4, a process was followed which was identical to that of Example 1, with the exception that in place of the phosphite antioxidant (A) (ADK STAB 517) which was used in Example 1, 8.0 parts of the phosphite antioxidant expressed by the Structural Formula (8) below (produced by Sumitomo Chemical Company, Limited: Sumilizer TNP) was used, and a recording medium was obtained.

The recording medium which was thus obtained was tested in the same manner as in Example 1, and  $\Delta E$  was measured. The results thereof are shown in Table 1.



## Comparative Example 5

In Comparative Example 5, a process was followed which was identical to that of Example 1, with the exception that in place of the phosphite antioxidant (A) (ADK STAB 517) which was used in Example 1, 8.0 parts of the phosphite antioxidant expressed by the Structural Formula (9) below (produced by Sumitomo Chemical Company, Limited: Sumilizer TPP-R) was used, and a recording medium was obtained.

The recording medium which was thus obtained was tested in the same manner as in Example 1, and  $\Delta E$  was measured. The results thereof are shown in Table 1.



## Comparative Example 6

In Comparative Example 6, a process was followed which was identical to that of Example 1, with the exception that in place of the phosphite antioxidant (A)

(ADK STAB 517) which was used in Example 1, 8.0 parts of the phosphite antioxidant expressed by the Structural Formula (10) below (produced by Sumitomo Chemical Company, Limited: Sumilizer P-16) was used, and a recording medium was obtained.

The recording medium which was thus obtained was tested in the same manner as in Example 1, and  $\Delta E$  was measured. The results thereof are shown in Table 1.



## Comparative Example 7

In Comparative Example 7, a process was followed which was identical to that of Example 1, with the exception that in place of the phosphite antioxidant (A) (ADK STAB 517) which was used in Example 1, 8.0 parts of the phosphite antioxidant expressed by the Structural Formula (11) below (produced by Sakai Chemical Industry Co., Ltd.: CHELEX-PC) was used, and a recording medium was obtained.

The recording medium which was thus obtained was tested in the manner as in Example 1, and  $\Delta E$  was measured. The results thereof are shown in Table 1.



## Comparative Example 8

In Comparative Example 8, a process was followed which was identical to that of Example 1, with the exception that in place of the phosphite antioxidant (A) (ADK STAB 517) which was used in Example 1, 8.0 parts of the phosphite antioxidant expressed by the Structural Formula (12) below (produced by Asahi Denka Kogyo K.K.: ADK STAB PEP-4C) was used, and a recording medium was obtained.

The recording medium which was thus obtained was tested in the same manner as in Example 1, and  $\Delta E$  was measured. The results thereof are shown in Table 1.



## Comparative Example 9

In Comparative Example 9, a process was followed which was identical to that of Example 1, with the exception that in place of the phosphite antioxidant (A) (ADK STAB 517) which was used in Example 1, 8.0 parts of the phosphite antioxidant expressed by the Structural Formula (13) below (produced by Asahi Denka Kogyo K.K.: ADK STAB 3010) was used, and a recording medium was obtained.

The recording medium which was thus obtained was tested in the same manner as in Example 1, and  $\Delta E$  was measured. The results thereof are shown in Table 1.

The recording medium which was thus obtained was tested in the same manner as in Example 1, and  $\Delta E$  was measured. The results thereof are shown in Table 1.



As is clear from Table 1, the color variation ( $\Delta E$ ) of the recording materials of Examples 1-18 was markedly smaller than that of Comparative Examples 1-9.

#### EXAMPLE 19

The coating fluid for the image receiving layer described hereinbelow was coated uniformly to the surface of white polyester film constituting the substrate used in Example 1, by means of an immersion method, and the solvent was volatilized, and subsequently, this was irradiated with ultraviolet rays by means of a high pressure mercury lamp, and an image receiving layer having a thickness of 5-6 micrometers was formed, and thus a recording medium was obtained.

| Coating Fluid for the Image Receiving Layer                                                                                                                                                                                      |           |
|----------------------------------------------------------------------------------------------------------------------------------------------------------------------------------------------------------------------------------|-----------|
| Polyester resin formed by the condensation polymerization of terephthalic acid/isophthalic acid/ethylene glycol/neopentyl glycol (molecular weight 15000-20000, glass transition temperature 67° C.)                             | 20 parts  |
| Polyester resin formed by the condensation polymerization of terephthalic acid/isophthalic acid sebacic acid/ethylene glycol/neopentyl glycol/1,4-butanediol (molecular weight 18000-20000, glass transition temperature 47° C.) | 50 parts  |
| Kayarad DPHA (Produced by Nippon Kayaku Co., Ltd.)                                                                                                                                                                               | 15 parts  |
| 2,2-bis (4-acryloyl oxydiethoxyphenyl) propane                                                                                                                                                                                   | 15 parts  |
| 1-hydroxycyclohexylphenyl ketone                                                                                                                                                                                                 | 3 parts   |
| Phosphite antioxidant expressed by Structural Formula (A) above (produced by Asahi Denka Kogyo K.K.: ADK STAB 517)                                                                                                               | 8.0 parts |
| Phenol compound expressed by Structural Formula (J) above (p-octyl phenol)                                                                                                                                                       | 3.9 parts |
| 2-hydroxy-4-octoxybenzophenone                                                                                                                                                                                                   | 4.8 parts |
| Bis (1,2,2,6,6-pentamethyl-4-piperidyl) sebacate                                                                                                                                                                                 | 4.8 parts |
| Silicon surfactant expressed by Structural Formula (S) above                                                                                                                                                                     | 0.5 part  |
| Methylethyl ketone                                                                                                                                                                                                               | 500 parts |
| Toluene                                                                                                                                                                                                                          | 100 parts |

The recording medium which was thus obtained was tested in the same manner as in Example 1, and  $\Delta E$  was measured. The results are shown in Table 2.

#### EXAMPLE 20

In Example 20, a process identical to that of Example 19 was followed, with the exception that in place of the two types of polyester resins which were used in Example 19, 70 parts of a polyester resin obtained by the condensation polymerization of terephthalic acid/isophthalic acid/ethylene glycol/neopentyl glycol/1,4-cyclohexane dimethanol (molecular weight 25,000-30,000, glass transition temperature 67° C.) was used, and the amount of the phosphite antioxidant (A) (ADK STAB 517) of Example 19 was set at a level of 6.5 parts, and the amount of the phenol compound (J) (p-octylphenol) which was used was set at a level of 3.2 parts, and a recording medium was obtained.

The recording medium which was thus obtained was tested in the same manner as in Example 1, and  $\Delta E$  was measured. The results thereof are shown in Table 2.

#### EXAMPLE 21

In Example 21, a process identical to that of Example 20 was followed, with the exception that the amount of the phosphite antioxidant (A) (ADK STAB 517) which was used was set at a level of 4.8 parts, and the amount of the phenol compound (J) (p-octylphenol) which was used was set at a level of 4.8 parts, and a recording medium was obtained.

10 The recording medium which was thus obtained was tested in the same manner as in Example 1, and  $\Delta E$  was measured. The results thereof are shown in Table 2.

#### EXAMPLE 22

15 In Example 22, a process identical to that of Example 20 was followed, with the exception that the amount of the phosphite antioxidant (A) which was used was set at a level of 3.2 parts, and the amount of the phenol compound (J) which was used was set at a level of 6.5 parts, and a recording medium was obtained.

The recording medium which was thus obtained was tested in the same manner as in Example 1, and  $\Delta E$  was measured. The results thereof are shown in Table 2.

#### EXAMPLE 23

20 In Example 23, a process identical to that of Example 20 was followed, with the exception that the amount of the phosphite antioxidant (A) which was used was set at a level of 1.6 parts, and the amount of the phenol compound (J) which was used was set at a level of 8 parts, and a recording medium was obtained.

25 The recording medium which was thus obtained was tested in the same manner as in Example 1, and  $\Delta E$  was measured. The results thereof are shown in Table 2.

#### EXAMPLE 24

30 In Example 24, a process identical to that of Example 20 was followed, with the exception that the amount of the phosphite antioxidant (A) which was used was set at a level of 6.5 parts, and the amount of the phenol compound (J) which was used was set at a level of 6.5 parts, and a recording medium was obtained.

35 The recording medium which was thus obtained was tested in the same manner as in Example 1, and  $\Delta E$  was measured. The results thereof are shown in Table 2.

#### EXAMPLE 25

40 In Example 25, a process identical to that of Example 20 was followed, with the exception that the amount of the phosphite antioxidant (A) which was used was set at a level of 8 parts, and the amount of the phenol compound (J) which was used was set at a level of 6.5 parts, and a recording medium was obtained.

45 The recording medium which was thus obtained was tested in the same manner as in Example 1, and  $\Delta E$  was measured. The results thereof are shown in Table 2.

#### EXAMPLE 26

50 In Example 26, a process identical to that of Example 19 was followed, with the exception that in place of the phosphite antioxidant (A) which was used in Example 19, 8.0 parts of the phosphite antioxidant expressed by Structural Formula (F) above (produced by Asahi Denka Kogyo K.K.: ADK STAB C) was used, and the amount of the phenol compound (J) which was used was set at a level of 1 parts, and a recording medium was obtained.

55 The recording medium which was thus obtained was tested in the same manner as in Example 1, and  $\Delta E$  was measured. The results thereof are shown in Table 2.

The recording medium which was thus obtained was tested in the same manner as in Example 1, and  $\Delta E$  was measured. The results thereof are shown in Table 2.

#### EXAMPLE 27

In Example 27, a process identical to that of Example 19 was followed, with the exception that in place of the phosphite antioxidant (A) which was used in Example 19, 8.0 parts of the phosphite antioxidant expressed by Structural Formula (F) above (produced by Asahi Denka Kogyo K.K.: ADK STAB C) was used, and the amount of the phenol compound (J) which was used was set at a level of 2.0 parts, and a recording medium was obtained.

The recording medium which was thus obtained was tested in the same manner as in Example 1, and  $\Delta E$  was measured. The results thereof are shown in Table 2.

#### EXAMPLE 28

In Example 28, a process identical to that of Example 19 was followed, with the exception that in place of the phosphite antioxidant (A) which was used in Example 19, 8.0 parts of the phosphite antioxidant expressed by Structural Formula (F) above (produced by Asahi Denka Kogyo K.K.: ADK STAB C) was used, and the amount of the phenol compound (J) which was used was set at a level of 3.9 parts, and a recording medium was obtained.

The recording medium which was thus obtained was tested in the same manner as in Example 1, and  $\Delta E$  was measured. The results thereof are shown in Table 2.

As is clear from Table 2, the recording materials of Examples 19-28, in which a phenol compound having the specified structure shown in Formula (4) above was used concurrently with the phosphite antioxidants having the specified structures shown in Formulas (1), (2), or (3) above, had color variances ( $\Delta E$ ) which were further reduced.

With respect to the recording materials of Examples 1-13, Comparative Examples 1-9, Examples 19-25, and Example 28, the magenta color of a VW-VS 100 color sheet for use in an NV-MP 1 video printer, produced by Matsushita Electric Industrial Co., Ltd., was used, and  $\Delta E$  was measured in the same manner as in the case of the cyan color of Example 1. The results thereof are shown in Tables 3 and 4.

As is clear from Table 3, with respect to the magenta color as well, the color variation ( $\Delta E$ ) of the recording materials of Examples 1-13, which contain phosphite antioxidants having the specified structures shown in the above Formulas (1), (2), and (3), was strikingly smaller than the  $\Delta E$  value of Comparative Examples 1-9. Furthermore, as is clear from Table 4, the color variation ( $\Delta E$ ) of the recording materials of Comparative Examples 19-25 and 28, which concurrently used phenol compounds having the specified structure shown in Formula (4) above was even smaller.

The recording density and dark fade out of the recording materials of Examples 8 and 20-25, which used the same dyeing resins, were measured according to the conditions below. The results thereof are shown in Table 5.

#### Recording Density

Recording was conducted using the cyan color of a VW-VS 100 color sheet for use in an NV-MP 1 video printer produced by Matsushita Electric Industrial Co., Ltd., and by means of a thermal head (950 ohms, 6

dots/ram) produced by Kyocera Corporation, under conditions such that the recording voltage was 13 V, and the pulse width was 14 msec. Subsequently, the reflection density of the recorded image was measured using a Macbeth densitometer (status A filter).

#### Dark Fade Out

Recording was conducted by means of a thermal head (950 ohms, 6 dots/mm) produced by Kyocera Corporation and using the cyan color of a VW-VS 100 color sheet for use in an NV-MP 1 video printer produced by Matsushita Electric Industrial Co., Ltd., under conditions such that the recording voltage was 15 V, and the pulse width was 10 msec. Subsequently, the recorded image was stored in a darkened area for a period of 7 days at a temperature of 60° C. and at a humidity of 60%; the reflection density of the image before and after storage was measured using a Macbeth densitometer (status A filter).

This dark fade out is shown in terms of a density residual rate (print %), which is calculated by means of the formula shown below. That is to say, when this numerical value approaches 100, this indicates that the density variation is small, and the dark fade out is good, while when the numerical value decreases, this indicates that the density is poor and the dark fade out is also poor.

density residual rate (%) =

$$\frac{\text{post-storage reflection density}}{\text{pre-storage reflection density}} \times 100$$

As is clear from Table 5, as the amount of the phenol compound shown in Formula (4) above which is added becomes large, the recording density of the recording medium becomes high, and the dark fade out of the recorded image is improved.

TABLE 1

| Number      | ANTIOXIDANT   | AMOUNT ADDED     | $\Delta E$ (CYAN) |
|-------------|---------------|------------------|-------------------|
| Example 1   | ADK STAB 517  | 8.0              | 10.6              |
| Example 2   | ADK STAB 1500 | 8.0              | 12.0              |
| Example 3   | ADK STAB 260  | 8.0              | 13.2              |
| Example 4   | ADK STAB 522A | 8.0              | 11.9              |
| Example 5   | JPP-613M      | 8.0              | 13.0              |
| Example 6   | ADK STAB 517  | 1.6              | 16.0              |
| Example 7   | ADK STAB 517  | 3.2              | 14.5              |
| Example 8   | ADK STAB 517  | 4.8              | 13.2              |
| Example 9   | ADK STAB 517  | 13.0             | 8.3               |
| Example 10  | ADK STAB 517  | 11.3             | 11.4              |
| Example 11  | ADK STAB C    | 8.0              | 11.6              |
| Example 12  | JPM-311       | 8.0              | 12.1              |
| Example 13  | JPM-313       | 8.0              | 12.3              |
| Example 14  | JPP-100       | 8.0              | 12.8              |
| Example 15  | ADK STAB C    | 1.6              | 16.0              |
| Example 16  | ADK STAB C    | 3.2              | 14.5              |
| Example 17  | ADK STAB C    | 13.0             | 10.2              |
| Example 18  | ADK STAB C    | 11.3             | 10.3              |
| Comparative | NONE          | —                | 20.0              |
| Example 1   | Comparative   | ADK STAB AO-75   | 8.0               |
| Example 2   | Comparative   | SUMILIZER BP-101 | 8.0               |
| Example 3   | Comparative   | SUMILIZER TNP    | 8.0               |
| Example 4   | Comparative   | SUMILIZER TPP-R  | 8.0               |
| Example 5   | Comparative   | SUMILIZER P-16   | 8.0               |
| Example 6   | Comparative   | CHELEX PC        | 8.0               |
| Example 7   | Comparative   | ADK STAB PEP-4C  | 8.0               |
|             |               |                  | 17.7              |

TABLE 1-continued

| Number                | ANTIOXIDANT       | AMOUNT ADDED | ΔE (CYAN) |
|-----------------------|-------------------|--------------|-----------|
| Example 8             | ADK STAB 3010 8.0 | 19.1         |           |
| Comparative Example 9 |                   |              |           |

TABLE 3-continued

| Number      | ANTIOXIDANT     | AMOUNT ADDED | ΔE (MAGENTA) |
|-------------|-----------------|--------------|--------------|
| Comparative | CHELEX PC       | 8.0          | 17.6         |
| Example 7   |                 |              |              |
| Comparative | ADK STAB PEP-4C | 8.0          | 17.9         |
| Example 8   |                 |              |              |

TABLE 2

| Number     | COMPOUND (A) | (AMOUNT ADDED) | COMPOUND (B)  | (AMOUNT ADDED) | ΔE (CYAN) |
|------------|--------------|----------------|---------------|----------------|-----------|
| Example 19 | ADK STAB 517 | (8.0)          | p-octylphenol | (3.9)          | 9.5       |
| Example 20 | ADK STAB 517 | (6.5)          | p-octylphenol | (3.2)          | 8.7       |
| Example 21 | ADK STAB 517 | (4.8)          | p-octylphenol | (4.8)          | 8.1       |
| Example 22 | ADK STAB 517 | (3.2)          | p-octylphenol | (6.5)          | 7.5       |
| Example 23 | ADK STAB 517 | (1.6)          | p-octylphenol | (8.0)          | 7.2       |
| Example 24 | ADK STAB 517 | (6.5)          | p-octylphenol | (6.5)          | 6.6       |
| Example 25 | ADK STAB 517 | (8.0)          | p-octylphenol | (6.5)          | 6.5       |
| Example 26 | ADK STAB C   | (8.0)          | p-octylphenol | (1.0)          | 9.9       |
| Example 27 | ADK STAB C   | (8.0)          | p-octylphenol | (2.0)          | 9.1       |
| Example 28 | ADK STAB C   | (8.0)          | p-octylphenol | (3.9)          | 7.7       |

TABLE 3

Comparative ADK STAB 3010 8.0 17.8

Example 9

| AMOUNT | ΔE (MA- |
|--------|---------|
|        |         |

TABLE 4

| Number     | COMPOUND (A) | (AMOUNT ADDED) | COMPOUND (B)  | (AMOUNT ADDED) | ΔE (MAGENTA) |
|------------|--------------|----------------|---------------|----------------|--------------|
| Example 19 | ADK STAB 517 | (8.0)          | p-octylphenol | (3.9)          | 6.6          |
| Example 20 | ADK STAB 517 | (6.5)          | p-octylphenol | (3.2)          | 6.8          |
| Example 21 | ADK STAB 517 | (4.8)          | p-octylphenol | (4.8)          | 4.9          |
| Example 22 | ADK STAB 517 | (3.2)          | p-octylphenol | (6.5)          | 5.8          |
| Example 23 | ADK STAB 517 | (1.6)          | p-octylphenol | (8.0)          | 5.7          |
| Example 24 | ADK STAB 517 | (6.5)          | p-octylphenol | (6.5)          | 3.3          |
| Example 25 | ADK STAB 517 | (8.0)          | p-octylphenol | (6.5)          | 3.0          |
| Example 28 | ADK STAB C   | (8.0)          | p-octylphenol | (3.9)          | 6.7          |

TABLE 5

| Number     | COMPOUND (A) | (AMOUNT ADDED) | COMPOUND (B)  | (AMOUNT ADDED) | PRINT DENSITY | DARK FADE OUT (%) |
|------------|--------------|----------------|---------------|----------------|---------------|-------------------|
| Example 8  | ADK STAB 517 | (4.8)          | NONE          |                | 0.97          | 91                |
| Example 20 | ADK STAB 517 | (6.5)          | p-octylphenol | (3.2)          | 1.15          | 92                |
| Example 21 | ADK STAB 517 | (4.8)          | p-octylphenol | (4.8)          | 1.25          | 94                |
| Example 22 | ADK STAB 517 | (3.2)          | p-octylphenol | (6.5)          | 1.38          | 97                |
| Example 23 | ADK STAB 517 | (1.6)          | p-octylphenol | (8.0)          | 1.54          | 98                |
| Example 24 | ADK STAB 517 | (6.5)          | p-octylphenol | (6.5)          | 1.50          | 94                |
| Example 25 | ADK STAB 517 | (8.0)          | p-octylphenol | (6.5)          | 1.46          | 93                |

| Number      | ANTIOXIDANT      | ADDED | GENTA) |
|-------------|------------------|-------|--------|
| Example 1   | ADK STAB 517     | 8.0   | 8.5    |
| Example 2   | ADK STAB 1500    | 8.0   | 12.4   |
| Example 3   | ADK STAB 260     | 8.0   | 13.4   |
| Example 4   | ADK STAB 522A    | 8.0   | 15.0   |
| Example 5   | JPP-613M         | 8.0   | 15.0   |
| Example 6   | ADK STAB 517     | 1.6   | 15.2   |
| Example 7   | ADK STAB 517     | 3.2   | 14.0   |
| Example 8   | ADK STAB 517     | 4.8   | 12.9   |
| Example 9   | ADK STAB 517     | 13.0  | 6.9    |
| Example 10  | ADK STAB 517     | 11.3  | 6.0    |
| Example 11  | ADK STAB C       | 8.0   | 8.9    |
| Example 12  | JPM-311          | 8.0   | 10.1   |
| Example 13  | JPM-313          | 8.0   | 10.0   |
| Comparative | NONE             | —     | 18.0   |
| Example 1   |                  |       |        |
| Comparative | ADK STAB AO-75   | 8.0   | 18.3   |
| Example 2   |                  |       |        |
| Comparative | SUMILIZER BP-101 | 8.0   | 25.2   |
| Example 3   |                  |       |        |
| Comparative | SUMILIZER TNP    | 8.0   | 16.8   |
| Example 4   |                  |       |        |
| Comparative | SUMILIZER TPP-R  | 8.0   | 16.6   |
| Example 5   |                  |       |        |
| Comparative | SUMILIZER P-16   | 8.0   | 19.7   |
| Example 6   |                  |       |        |

What is claimed is:

1. A recording medium for sublimation heat-sensitive transfer recording, wherein an image receiving layer comprising a resin composition containing dyeable resin and at least one member selected from the group consisting of phosphite antioxidants shown in Formulas (1), (2), and (3) below, is formed on a substrate

55



60 65 where R<sub>1</sub> and R<sub>2</sub> represent H or an alkyl group having a number of carbon atoms within a range of 1-20, R<sub>3</sub> and R<sub>4</sub> represent an alkyl group having a number of carbon atoms within a range of 1-20, X represents H or

an atomic group having 1-10 carbon atoms as a main skeleton thereof, and n has a value of 1, 2, 3, or 4



wherein R<sub>5</sub> and R<sub>6</sub> represent H or an alkyl group having a number of carbon atoms within a range of 1-20, R<sub>7</sub> represents an alkyl group having a number of carbon atoms within a range of 1-20, Y represents H or an atomic group having 1-10 carbon atoms as a main skeleton thereof, and n has a value of 1, 2, 3, or 4.



wherein R<sub>8</sub>, R<sub>9</sub>, R<sub>10</sub>, and R<sub>11</sub> represent H or an alkyl group having a number of carbon atoms within a range of 1-20, Z represents H or a monocyclic atomic group having 1-13 carbon atoms as a main skeleton thereof, and n has a value of 1, 2, 3, or 4.

2. A recording medium for sublimation heat-sensitive transfer recording according to claim 1, wherein said resin composition constituting said image receiving layer furthermore contains at least one member selected from the group of phenol compounds shown in Formula (4) below



wherein R<sub>12</sub>, R<sub>13</sub>, and R<sub>14</sub> represent H or an alkyl group having a number of carbon atoms within a range of 1-4.

3. A recording medium for sublimation heat-sensitive transfer recording according to claim 1 or claim 2, wherein said resin composition constituting said image receiving layer contains polyester resin as at least one component of said dyeable resin.

4. A recording medium for sublimation type heat-sensitive transfer recording according to claim 1 or claim 2, wherein said resin composition constituting said image receiving layer contains at least one cross-linking component.

5. A recording medium for sublimation heat-sensitive transfer recording according to claim 4, wherein the amount of said cross-linking component is such that with respect to a total amount of said dyeable resin and said cross-linking component of 100 parts by weight, said dyeable resin is present in an amount of 40-95 parts by weight, while said cross-linking component is present in an amount of 60-5 parts by weight.

6. A recording medium for sublimation heat-sensitive transfer recording according to claim 4, wherein the

amount of said at least one member selected from the group consisting of compounds shown in Formulas (1), (2), and (3) is such that, with respect to a total amount of said dyeable resin and said cross-linking component constituting said image receiving layer of 100 parts by weight, said component is present in an amount of 0.3-20 parts by weight.

7. A recording medium for sublimation heat-sensitive transfer recording according to claim 4, wherein the amount of said at least one member selected from the group consisting of compounds shown in Formulas (1), (2), and (3) is such that, with respect to a total amount of said dyeable resin and said cross-linking component constituting said image receiving layer of 100 parts by weight, said component is present in an amount of 1-15 parts by weight.

8. A recording medium for sublimation heat-sensitive transfer recording according to claim 4, wherein the amount of said at least one member selected from the group consisting of compounds shown in Formula (4) is such that, with respect to a total amount of said dyeable resin and said cross-linking component constituting said image receiving layer of 100 parts by weight, said compound is present in an amount of 0.3-20 parts by weight.

9. A recording medium for sublimation heat-sensitive transfer recording according to claim 4, wherein the amount of at least one member selected from the group consisting of compounds shown in Formula (4) is such that, with respect to a total amount of said dyeable resin and said cross-linking component constituting said image receiving layer of 100 parts by weight, said compound is present in an amount of 1-15 parts by weight.

10. A recording medium for sublimation heat-sensitive transfer recording according to claim 2, wherein the amount of said at least one member selected from the group consisting of compounds shown in Formula (4) is such that, with respect to 100 parts by weight of said dyeable resin constituting said image receiving layer, said component is present in an amount of 0.3-20 parts by weight.

11. A recording medium for sublimation heat-sensitive transfer recording according to claim 1, wherein the amount of said at least one member selected from the group consisting of compounds shown in Formulas (1), (2), and (3) is such that, with respect to a total amount of said dyeable resin constituting said image receiving layer of 100 parts by weight, said compound is present in an amount of 0.3-20 parts by weight.

12. A recording medium for sublimation heat-sensitive transfer recording according to claim 1, wherein the amount of said at least one member selected from the group consisting of compounds shown in Formulas (1), (2), and (3) is such that, with respect to a total amount of said dyeable resin constituting said image receiving layer of 100 parts by weight, said component is present in an amount of 1-15 parts by weight.

13. A recording medium for sublimation heat-sensitive transfer recording according to claim 1, wherein the amount of said at least one member selected from the group consisting of compounds shown in Formula (4) is such that, with respect to 100 parts by weight of said dyeable resin constituting said image receiving layer, said compound is present in an amount of 1-15 parts by weight.

14. A recording medium for sublimation heat-sensitive transfer recording as claimed in claim 1, wherein

said resin composition contains a phosphite antioxidant of Formula (1).

15. A recording medium for sublimation heat-sensitive transfer recording as claimed in claim 1, wherein said resin composition contains a phosphite antioxidant of Formula (2).

16. A recording medium for sublimation heat-sensitive transfer recording as claimed in claim 1, wherein said resin composition contains a phosphite antioxidant of Formula (3), wherein n in Formula (3) is 2, 3 or 4.

17. A recording medium for sublimation heat-sensitive transfer recording as claimed in claim 1, wherein said resin composition contains a phosphite antioxidant of Formula (3), wherein, in Formula (3) Z is H.

18. A recording medium for sublimation heat-sensitive transfer recording as claimed in claim 1, wherein in Formula (3) Z is H, —C<sub>8</sub>H<sub>17</sub>, 13 C<sub>10</sub>H<sub>21</sub> or —C<sub>13</sub>H<sub>27</sub>.

19. A recording medium for sublimation heat-sensitive transfer recording as claimed in claim 1, wherein said resin composition contains at least one member selected from the group consisting of



(A)

35

and



(B)

40

20. A recording medium for sublimation heat-sensitive transfer recording as claimed in claim 1, wherein said resin composition contains at least one member selected from the group consisting of

45

55

60

65



(C)



(D)

and



(E)



(F)



(G)



(H)



(I)

\* \* \* \* \*

UNITED STATES PATENT AND TRADEMARK OFFICE  
**CERTIFICATE OF CORRECTION**

PATENT NO. : 5,326,741  
DATED : July 5, 1994  
INVENTOR(S) : Kenji Kishi, et al

It is certified that error appears in the above-identified patent and that said Letters Patent is hereby corrected as shown below:

Column 23, Claim 1, line 31, delete "monocyclic" and insert --non-cyclic--.

Signed and Sealed this  
Nineteenth Day of September, 1995

Attest:



*Attesting Officer*

BRUCE LEHMAN

*Commissioner of Patents and Trademarks*